

## UNITED STATES PATENT OFFICE

2,093,031

PRODUCT AND METHOD AND COMPOSITION  
FOR CADMIUM-TIN ALLOY PLATINGLeroy Camel, Maple Heights, Ohio, assignor to  
The Plating and Galvanizing Company, Cleve-  
land, Ohio, a corporation of OhioNo Drawing. Application April 1, 1937,  
Serial No. 134,425

## 6 Claims. (CL 204—1)

This invention, as indicated, relates to a method and composition for cadmium-tin alloy plating, especially in relation to ferrous articles. More particularly, it comprises a composition having a combination of elements adapted to bring about bright plating of cadmium-tin alloy, resulting in a new product, and providing a method adaptable for quantity production with a product of uniform quality and dependable finish. The invention especially includes the plating of ferrous articles with an alloy of cadmium and tin, the tin being present in relatively small amount, but being effective in conjunction with the other elements employed in producing a bright cadmium-tin alloy coating comparable with platings produced through the use of special brightening agents which are not alloyed.

Various types of cadmium plating compositions and processes are known, but many of these are not adapted for commercial use either because of cost or intricacy of handling, or by reason of difficulty in maintaining uniformity of product. Heretofore the use of tin and elements associated with the tin group have been referred to as having a detrimental effect in the cadmium bath, tin being described as "analogous to the 'poisoning' effect of arsenic in other catalytic operations."

The present invention utilizes a cyanide bath as the electrolyte and includes with the same, small quantities of compounds to improve the conductivity of the bath and to bring about a bright coating upon the articles being plated. It has been found that the cyanide bath in general results in the best quality of color for the product, but in many instances the time factor of the operation has been poor or the control of the operation has been difficult. With the composition herein described, it has been found that a uniformly high rate of production can be maintained, and a durable coating of a cadmium-tin alloy deposit of high lustre can be maintained on the product, with no unfavorable factors to be taken into account as to the maintenance of the bath or excessive cost or complication in carrying out the process.

The process, while adapted to be carried out in certain proportionate relations between the elements entering into the same, is by no means restricted to certain critical proportions, but has a reasonable range of limits as to quantities, as well as to substitution of equivalent elements. It is pointed out, however, that the amount of tin used must be maintained at a very small amount, whether the tin is introduced into the

solution in the form of various compounds of such element, or as a portion of the anode.

The preferred formula for producing the electrolyte comprises the following:

|                  |                       |     |
|------------------|-----------------------|-----|
| Sodium cyanide   | oz. per gal. of water | 16  |
| Cadmium oxide    | do                    | 5   |
| Tin oxide        | g. per gal. of water  | 0.2 |
| Glue (.88 oz.)   | cc. per gal. of water | 25  |
| Sodium hydroxide | oz. per gal. of water | 3   |
| Water            | gal.                  | 10  |

As has been stated, some latitude of proportions is permissible, as well as certain substitution of equivalents, but the amount of tin oxide or other source of tin for the electrolyte must be kept closely to the lower limits, inasmuch as an excess of tin results in a deposit of a spongy character which cannot be maintained under severe conditions of use and which will not be of a bright finish. When the amount of tin is kept at approximately the amount stated in the formula above set forth, the resulting plating is not only as bright as can be obtained through the use of various brightening agents, such as sulphonated oils and the like, but is of a more tenacious character, and corrosion effects on the coating are avoided for a much longer period.

If desired, a mixture in dry form of all the ingredients, including the glue in granulated form, may be prepared in a single package, and upon the addition of such ingredients to a water bath, which may be very moderately heated to assist in the speed of dissolution of the powdered and granular material, the bath will be ready for use.

The bath, when fully prepared, will be found to permit the use of current up to 45 amperes in the plating circuit, or as low as 10 amperes per square foot of surface at preferably from 3 to 5 volts.

The anode utilized preferably comprises a composition of pure cadmium and tin in the relative amounts which would be found in a bath prepared in accordance with the formula. However, an anode of pure cadmium may be utilized with the tin present in the solution, or an anode partially formed of cadmium with or without tin associated therewith, and may be utilized with non-metallic anodes.

At a temperature of between 60 and 90 degrees Farenheit, the plating bath above set forth will coat ferrous articles with a smooth tenacious coating of cadmium-tin alloy in approximately from 4 to 6 minutes, and such coating will be of

fine grain and bright texture, and have great durability and resistance to corrosion.

When articles are plated with the cadmium-tin alloy as above outlined, they may be used for many purposes without any finishing treatment, such as buffing or the like. The coating referred to is also adapted to form a base coating upon which some other metals, such as nickel or chrome, may be deposited with an unusually bright and hard finished effect.

Other modes of applying the principle of my invention may be employed instead of those explained, change being made as regards the means and steps herein disclosed, provided the means stated by any of the following claims or the equivalent of such stated means be employed.

I therefore particularly point out and distinctly claim as my invention:

1. The process of producing bright smooth coatings of cadmium-tin alloy on ferrous articles, which includes the step of adding to a cyanide electrolytic bath in addition to the cadmium an amount of tin not in excess of 0.2 grams per gallon of electrolyte to serve as an alloy with the cadmium.

2. The process of cadmium-tin alloy plating in a cyanide bath which comprises the electroplating of cadmium with an amount of tin associated therewith, the cadmium being in the form of an oxide in the proportion of 5 ounces per gallon of water, and the tin being in the form of an oxide in the proportion of 0.2 grams per gallon of water.

3. The process of cadmium-tin alloy plating which comprises the electroplating of cadmium from a cyanide bath containing cadmium oxide, and tin oxide in concentration in the order of 0.2 grams to the gallon in the presence of sodium hydroxide, and animal glue as a colloidal brightening agent.

4. In a cadmium tin cyanide bath for electroplating, the combination of sodium cyanide to the amount of 16 ounces per gallon of water, cadmium oxide to the amount of 5 ounces per gallon of water, tin oxide to the amount of 0.2 grams per gallon of water, glue to the amount of 25 cubic centimeters per gallon of water, and sodium hydroxide to the amount of 3 ounces per gallon of water.

5. A composition of matter adapted for use in forming an electrolyte for the electrodeposition of a cadmium-tin alloy on ferrous articles, consisting for each gallon of water to be used of dry pulverized and granular material in the proportion of 16 ounces of sodium cyanide, 5 ounces of cadmium oxide, 0.2 grams of tin oxide, .88 ounces of glue, and 3 ounces of sodium hydroxide.

6. As a new article of manufacture, a metal article having an electrolytic coating comprising an alloy of cadmium and tin produced by the process of electrodepositing said coating from a cadmium cyanide electrolytic bath containing in addition to the cadmium oxide an amount of tin oxide not in excess of 0.2 grams per gallon of electrolyte to serve as an alloy with the cadmium.

LEROY CAMEL.